

(No Model.)

E. B. STOCKING.

METHOD OF REDUCING OLD RAILROAD RAILS TO PLATES.

No. 339,118.

Patented Mar. 30, 1886.



WITNESSES:

*L. B. Mills*  
*Wm. Duvall*

INVENTOR

*E. B. Stocking*

# UNITED STATES PATENT OFFICE.

EDGAR B. STOCKING, OF WASHINGTON, DISTRICT OF COLUMBIA.

## METHOD OF REDUCING OLD RAILROAD-RAILS TO PLATES.

SPECIFICATION forming part of Letters Patent No. 339,118, dated March 30, 1886.

Application filed February 18, 1886. Serial No. 192,338. (No model.)

*To all whom it may concern:*

Be it known that I, EDGAR B. STOCKING, a citizen of the United States, residing at Washington, in the District of Columbia, have invented certain new and useful Improvements in the Method of Reducing Old Railroad-Rails to Plates, of which the following is a specification, reference being had therein to the accompanying drawings.

10 My invention relates to an improved method of reducing railroad-rails and other forms of metal having lateral projections at opposite edges to plate metal, the object of my invention being to avoid forcing any of the material forming the head or flange of the rail or rail-section over onto the web of said rail or rail-section, so that the plates produced from the rail-sections shall be free from "cold-shuts" and overlapping non-welded fibers, in order

15 20 that the plates produced shall be homogeneous and adapted for the production of nails and other articles in which the fibers or grain of the metal shall be uniform, compact, and longitudinally disposed in said articles.

25 Heretofore old rails have been cut into pieces or sections of about three feet in length, which have been heated to a proper working-point and passed longitudinally through suitable rolls for reducing to a certain extent the lateral dimensions of the head and flange of the rail-section, and then the rail-section or blank has been passed edgewise through plain rollers to further reduce the lateral dimensions of the head and flange portions thereof, 30 and finally, by passing the blank longitudinally through plain rollers, the blank has been reduced to plate form of the desired thickness.

In the second step of the method above set forth as having heretofore been practiced—40 namely, the edgewise rolling of the blank or rail section—a part of the head or of the flange portion is forced over onto the web portion of the same, producing what is known as a "cold-shut" or non-welded overlap in the blank. It has been attempted to overcome 45 this defect by performing the edgewise rolling in rolls of unequal diameters, and by reversing the blank between succeeding passes of the same through said rolls; but, even by the use 50 of such rolls and reversals, there will be found evidences of a slight crowding of the metal

over onto the web, the metal of the head portion of the blank being slightly forced onto the web on one side of the rail section or blank, and the metal of the flange portion of the blank being slightly forced over onto the web on the other side of the section or blank, so that several double passes of the blank through such rolls are required, together with reversals of the blank, whereby the edge of 55 the blank that last emerged from the rolls in one double pass shall be the first to enter the rolls in the next succeeding double pass, in order that the overlap produced by one pass may be rolled back in the succeeding pass or 60 65 passes.

By my improved step in the method of reducing old rails to plate I do not produce any overlapping of either the head or flange portion of the blank upon the web, and therefore 70 any subsequent rolling of any overlap from the web is not required; so that a better product is secured, and this by a less number of passes of the blank through the rolls. My improved step consists in commencing the 75 edgewise rolling of the rail-section or of the blank at or upon the web, as will hereinafter be more specifically described.

It is apparent that after a rail-section has been longitudinally rolled, so as to reduce the 80 lateral dimensions of its head and flange as much as possible without forcing any of the material of either upon the web, (preliminary longitudinal rolling having long been practiced in the art,) any subsequent edgewise rolling 85 which takes effect at either edge of the blank must force more or less of the material of the advancing edge upon the web, and the object of my invention is to avoid this result, and this I accomplish by beginning the edgewise 90 rolling at or upon the web portion of the blank and thus compress, draw out, or roll down only the following portion of the blank in the direction of its movement through the rolls. By this improved step it may be said 95 that I pass through the rolls the advancing edge of the blank without compressing it at the time of or during that passage of the blank in which the following edge of the blank is compressed, rolled, or drawn out; or, in other 100 words, I reduce either the head or flange portion of the blank by beginning the reduc-

tion at or upon the web, and thus I reduce both the head and the flange without forcing either upon the web, as both are reduced by rolling or drawing them in a direction away from the web. All of these results are the consequence of commencing the reduction at or upon the web.

I have in the accompanying drawings illustrated several different kinds of mechanism for carrying out my invention, and although I do not limit the same to any particular mechanism for its practice, yet for the purpose of rendering my invention clear to persons skilled in the art reference is had to the said drawings, in which—

Figure 1 is a cross-section of an ordinary railroad-rail. Fig. 2 is the form herein designated as the blank, the same being shown in cross-section. Fig. 3 is a like view of the same blank after one of the edges of the same has been reduced. Fig. 4 is a like view of the same after both the head and flange portions have been reduced. Fig. 5 represents the blank in section, and in position between two rolls for the reduction of its flange portion. Fig. 6 is a plan of the finished plate, the dotted lines indicating the usual manner of forming nails therefrom. Fig. 7 is a side elevation of a set of "three-high" rolls adapted to reduce rail-sections to plates according to my method. Fig. 8 is a vertical section on the line 1 of Fig. 7. Figs. 9, 10, and 11 are modified forms of mechanism adapted to practice my method.

Like letters refer to like parts in all the figures, and the straight arrows indicate the direction in which the material passes through the rolls, and the curved arrows indicate the direction of rotation of the rolls.

A represents the head portion; B, the web portion, and C, the flange portion of a rail or rail-section. The rail-section is first passed longitudinally through between the rolls D E at F, and then through between the rolls E and G at H, for the purpose of reducing the lateral dimensions of the head A and flange C thereof, until the same shall approximate or assume substantially the form shown in Fig. 2, which form I denominate a blank. In this instance the rolls D and E are cut away, as at D' E', in order to permit of the insertion of the head portion A, or flange portion C, edgewise between the rolls without compressing, rolling, or drawing the same, and in order that after the same shall have been inserted, the unremoved portion of the rolls D and E may commence their action at or upon the following flange or head portion of the blank and compress, roll, draw, or reduce the same in a direction away from the web as the blank continues its passage through the rolls. Instead of cutting away portions of both rolls, D and E, a portion may be removed from only one of a pair of rolls, as shown in Fig. 11, and, as shown in Fig. 9, a portion need not be removed from either roll.

The construction illustrated in Fig. 9 consists in mounting each of the rolls eccentrically—that is, the shafts or bearings E<sup>2</sup> D<sup>2</sup> of the rolls D and E are eccentric—so that the point of the periphery of each of the rolls which is at its longest radius travels in the direction of the dotted line X, whereby, during each revolution of the rolls, the space between them varies from that shown in full lines to that shown by the dotted lines Y. Now, it will be seen that during each revolution of the rolls sufficient space exists between them through which the head or flange portion of the blank may pass without being acted upon by the rolls, in order that the following head or flange portion may be compressed, rolled, or drawn out in a direction from the web portion thereof.

In Fig. 10 the rolls D and E are mounted in a frame, I, which is open, as at I', at one end of the rolls, and the roll D is mounted in a vertically-reciprocating frame, D<sup>2</sup>, adapted to be raised and lowered by a lever, D<sup>3</sup>, pivoted to the frame I at D<sup>4</sup>, so that the roll D may be moved up to or dropped away from the roll E, as shown in dotted lines in said figure, in order to permit of the passage of the head or the flange portion of a blank edgewise through the rolls without being acted upon thereby until the web portion of the blank is between the rolls, when the operator depresses the lever D<sup>3</sup>, and this elevates the roll D, so that the following head or flange portion of the blank shall be operated upon.

The opening I' of the frame-work allows the passage of either a portion of the blank or of any tools for guiding the same through the rolls, although it is apparent that the lever D<sup>3</sup> may be arranged at the front of the machine and the frame-work I be complete, and the blank passed edgewise through between the rolls, as in the preceding operations described.

In Fig. 11 a roll, E, with the cut-away portion or recess E', is arranged at the top of the series of rolls. A plain roll, D, is arranged at the middle, and a similar roll, C, at the bottom. A table, J, may be arranged in front of the bite of the rolls D and E, to assist in presenting the blank to the cut-away portion of the roll E, so that only the following edge or flange of the blank shall be operated upon by the rolls D and E, when said blank takes the direction indicated by the arrows and falls upon a return-table, K, which is inclined so as to direct said blank into the bite of the rolls D and C, from which it emerges with its following or head portion drawn out in a direction from its web portion, after which it is rolled longitudinally to a proper thickness to form a plate for a desired purpose—as, for instance, said plate being subsequently cut, as indicated by the dotted lines Z, to form nails, (see Fig. 6,) the portions A, B, and C in said figure indicating, respectively, the head, web, and flange portions of the material.

Other modified arrangements of mechanical

devices can be readily devised for practicing my invention; but, as before stated, I do not limit the same to any particular mechanism, and I should deem the provision of other means than those herein shown and described for the preliminary reduction of the rail-section to a desired form of blank, and for the passage of the advancing edge of such blank through and between rolls without compression of the same, as still being mechanism adapted to practice my invention.

Having described my invention and mechanism for practicing the same, what I claim is—

15 1. A step in a method of reducing old rails to plates, which consists in commencing the

edgewise rolling at or upon the web, substantially as specified.

2. The method of reducing old rails to plates, which consists in, first, preliminarily reducing 20 the head and flange portions of the rail to form a blank; second, rolling said blank edgewise, commencing said rolling at or upon the web; and, third, rolling said blank longitudinally to reduce it to a proper thickness, substantially as specified. 25

In testimony whereof I affix my signature in presence of two witnesses.

EDGAR B. STOCKING.

Witnesses:

WM. S. DUVALL,  
LOUIS C. HILLS.